

Dec. 4, 1962

E. L. DUNN ET AL

3,067,030

NICKEL BASE ALLOY

Filed Aug. 13, 1958

2 Sheets-Sheet 1

Fig 1

AVERAGE STRESS RUPTURE DATA FOR CAST ALLOYS



INVENTORS:  
EUGENE L. DUNN  
JAMES E. WILSON  
MARION E. CIESLICKI  
JOSEPH B. MOORE

BY *Lee H. Schles*  
ATTORNEY—

Fig 2

Dec. 4, 1962

E. L. DUNN ET AL

3,067,030

NICKEL BASE ALLOY

Filed Aug. 13, 1958

2 Sheets-Sheet 2



# United States Patent Office

3,067,030

Patented Dec. 4, 1962

## 1

3,067,030

### NICKEL BASE ALLOY

Eugene Ludwick Dunn, Batavia, and James Ellis Wilson, Loveland, Ohio, and Marion Edward Cieslicki, Worcester, and Joseph Burton Moore, Westboro, Mass., assignors, by mesne assignments, to the United States of America as represented by the Secretary of the Air Force

Filed Aug. 13, 1958, Ser. No. 754,364  
1 Claim. (Cl. 75—171)

This invention relates to precipitation hardening type, vacuum melted nickel base alloys and to their heat treatment, the alloys being especially suitable for use in the casting of articles and for elevated temperature applications under stressed conditions.

The best nickel base alloys developed heretofore for high temperature, high stressed conditions such as may be experienced by cast blades, vanes, buckets or struts in gas turbine apparatus, tend to lose some of their strength properties at a substantially increasing rate in the 1600° F. and above range. At 1800° F. and above, articles such as blades made from the best of such known alloys have failed in relatively short periods of time under only moderately stressed conditions such as 15,000 pounds per square inch.

It is well known that the structure of many alloys, including nickel base alloys, is composed of a group of grains joined at grain boundary areas between the grains. At low temperatures, the grain boundary is more resistant to stress than the grains; therefore failure occurs through the grains or transgranularly. However, at elevated temperatures the grain boundaries can become more plastic and tend to allow the grains to slip over one another causing failure between the grains or intergranularly. Therefore, in order to strengthen nickel base alloys for elevated temperature applications, it is necessary to place hard, "blocking" particles in the grain boundaries to prevent such slipping.

It is believed that nickel base alloys for high temperature applications are hardened through the precipitation of a phase called "gamma prime" sometimes referred to as  $Ni_3(Al, Ti)$  in which it is seen that the elements aluminum and titanium are significant. In addition, hard particles of carbides and borides strategically precipitated or located in the grain boundaries affect the high temperature strength of such alloys. When particles such as these are deposited or precipitated, the alloy is called a "precipitation hardening" type of alloy.

Besides the elements boron and carbon which cooperate to form the borides and carbides, the element molybdenum cooperates to add solution strengthening to nickel base alloys. Therefore, although the elements aluminum, titanium, boron and molybdenum have been included in other known nickel base alloys, their interactions in certain narrow ranges, coupled with the effects of heat treatment and size of metal grains, has not previously been clearly defined.

An object of this invention is to provide an improved, precipitation hardening type, vacuum melted nickel base alloy and heat treatment for that alloy so as to produce a material suitable for use in the casting of articles and characterized by the fact that it has improved strength properties under stress conditions at elevated temperatures.

Briefly stated in accordance with one aspect of our invention, we provide an improved, precipitation hardening type vacuum melted nickel base alloy including the important elements titanium, aluminum, boron and molybdenum in percent by weight of 3—4 titanium, 0.05—0.10 boron, 3.6—5.0 aluminum and 4—7 molybdenum. In gen-

## 2

eral our alloy comprises in percent by weight up to about 0.08 carbon, about 4—6 iron, about 14—17 chromium, about 3—4 titanium, about 0.05—0.10 boron, about 3.6—5.0 aluminum, about 4—7 molybdenum, with the balance essentially nickel and impurities. In cast form our alloy, though relatively strong in the as-cast condition, may be further strengthened through heat treatment by first heating within the range of 2075—2200° F. and then air cooling. We have found that the average grain diameter of our cast alloy is a significant factor in determining strength properties. We prefer the average grain diameter of our alloy to be in excess of 0.015 inch.

The composition range of our alloy and its heat treatment will be better understood from our description taken in conjunction with the accompanying drawings and the following examples which are given by way of illustration only and not in any way by limitation. The scope of our invention will be pointed out in the claims.

In the drawings:

FIGURE 1 is a graph of the curves which compare stress rupture strength of our alloy in cast and heat treated form with other currently available elevated temperature cast alloys;

FIGURE 2 is a graph showing the tensile and yield strengths of our alloy in cast and heat treated form as well as percent reduction of area and elongation;

FIGURE 3 is a graph comparing stress rupture life to average grain diameter.

The chemical compositions of the best available alloys suitable for use at elevated temperatures are shown in Table 1 along with the chemical composition of our alloy in our preferred range. Included in these alloys as impurities may be, in percent by weight, a maximum of about 0.1 manganese, about 0.1 silicon, about 0.01 sulfur and about 0.01 copper.

Table 1  
[Composition in percent by weight]

|    | Our Alloy | Alloy B  | Alloy B | Alloy C  | Alloy D |
|----|-----------|----------|---------|----------|---------|
| C  | .08 max.  | .10—.20  | .02     | .20 max. | .1 max. |
| Fe | 4—6       | 3.5—5.0  | 0       | 5        | 2       |
| Cr | 14—16     | 14—17    | 15      | 11—14    | 18      |
| Ti | 3.25—3.65 | 2.0—3.0  | 0       | .25—1.25 | 3       |
| B  | .07—.09   | 0        | 0.1     | 0        | 0       |
| Al | 4.4—4.8   | 3.25—4.0 | 6.6     | 5.5—6.5  | 3       |
| Mo | 4.5—6.0   | 4.5—6.0  | 5       | 3.5—5.5  | 4       |
| Co | 0         | 0        | 0       | 0        | 18      |
| Cb | 0         | 0        | 0       | 2        | 0       |
| Ni | Bal.      | Bal.     | Bal.    | Bal.     | Bal.    |

Two of the tests generally conducted on alloys to determine their physical properties are called "stress rupture" and "tensile" tests. The results of these tests are reported as "stress rupture strength" and "tensile strength" respectively and are generally defined as follows:

"Stress rupture strength" is the value of stress in pounds per square inch obtained by dividing the amount of an applied load by the area supporting that load initially while the test specimen is maintained at a selected temperature. The strength of material of a test specimen is also measured by the length of time it resists failure at a given stress and temperature. Such a length of time is called "stress rupture life." By incorporating such values as temperature, initially applied load and stress rupture life into a special graph, later to be described, that graph may be used to predict the life of a material or the time a given material can be expected to be operable prior to failure under a specified stress and at a specified temperature.

"Tensile strength," sometimes called "ultimate strength," is the value in pounds per square inch obtained when the maximum load recorded during the straining of a speci-

men is divided by the cross-sectional area of the specimen before straining.

Referring to FIGURE 1 stress rupture strengths are represented by the comparison of stress with a time-temperature parameter shown at the horizontal coordinate. This parameter, known as the Larson-Miller Parameter, has been calculated from the formula  $P = T(20 + \log t) \times 10^{-3}$  in which  $P$  equals the time-temperature parameter number,  $T$  equals absolute temperature in degrees Rankine and  $t$  equals the time in hours. The curves of FIGURE 1 have been prepared from a large amount of stress rupture test results and represent a compact summary of a wide range of data. Using this special graph it is possible to predict the stress rupture life of a material under a given load at a given temperature.

5

10

15

properties. Metallurgical technology along these lines has advanced to the point where it is no longer possible to broadly designate the composition range of such elements as aluminum, titanium, molybdenum and boron and still be able to predict the physical properties which will result. In addition, new important heat treatment cycles must be specified in order to control the precipitation of phases which are developed in alloys having aluminum, titanium, molybdenum and boron as part of their composition.

As an illustration, Table 3 includes the composition ranges and the average stress rupture life of a number of heats of material which we have prepared and tested. The stress rupture properties were obtained at 1800° F. with the samples under an axial load of 15,000 pounds per square inch:

Table 3

[Composition (percent by weight)]

| Ex.      | Avg.<br>Stress<br>Rupture<br>Life<br>(Hours) | C   | Fe  | Cr   | B   | Ti  | Al  | Mo  | Ni   | Si  | Mn  | S    |
|----------|----------------------------------------------|-----|-----|------|-----|-----|-----|-----|------|-----|-----|------|
| A-2----- | 94                                           | .05 | 4.8 | 15.6 | .09 | 2.1 | 4.6 | 4.0 | Bal. | .10 | .05 | .006 |
| A-3----- | 213                                          | .05 | 4.8 | 15.6 | .09 | 2.8 | 4.6 | 4.0 | Bal. | .10 | .05 | .005 |
| A-4----- | 290                                          | .05 | 4.8 | 15.0 | .09 | 3.5 | 4.6 | 4.0 | Bal. | .10 | .05 | .005 |
| G-3----- | 313                                          | .08 | 4.8 | 15.6 | .09 | 4.0 | 3.6 | 6.9 | Bal. | .06 | .05 | .006 |
| C-3----- | 543                                          | .05 | 4.7 | 15.2 | .08 | 3.5 | 4.4 | 5.3 | Bal. | .10 | .05 | .007 |
| C-1----- | 59                                           | .07 | 4.7 | 15.8 | .08 | 3.5 | 2.6 | 5.3 | Bal. | .10 | .05 | .007 |
| D-4----- | 446                                          | .07 | 4.8 | 14.8 | .08 | 2.7 | 4.5 | 5.4 | Bal. | .06 | .05 | .007 |

It is to be noted that our alloy in vacuum cast form when heat treated according to Example A shown in Table 6 herein, and having an average grain diameter greater than .015 inch has stress rupture strength properties superior to any other available high temperature nickel base alloy. When heat treated according to Example C of Table 6, our alloy in vacuum cast form is shown to have even greater stress rupture strength. These increased strengths are attributed not only to the special heat treatments as later herein described, but also to the special ranges of titanium, boron, aluminum and molybdenum as well as the specification of average grain diameter in excess of about 0.015 inch.

Although Alloy A of Table 1 has a range of elements which might at first appear to be similar to that of our alloy, reference to FIGURE 1 shows that the differences in the amounts of aluminum, boron, titanium and carbon combine with other elements and phases to result in a much weaker alloy than is ours.

Figure 2 represents the average of results of tensile testing of our alloy of the following broad composition range, vacuum melted, vacuum cast and heat treated according to Example A of Table 6:

Table 2

[Composition in percent by weight]

|          |       |          |           |
|----------|-------|----------|-----------|
| C -----  | 1.08  | B -----  | 0.05-0.10 |
| Fe ----- | 4-6   | Al ----- | 3.6-5.0   |
| Cr ----- | 14-17 | Mo ----- | 4-7       |
| Ti ----- | 3-4   | Ni ----- | Balance   |

1 Max.

In addition to showing the ultimate strength of our improved alloy, FIGURE 2 summarizes a large amount of data to report the ductility of our alloy in terms of the reduction in area and elongation of the sample bar during testing. The term "0.2% yield strength" shown in FIGURE 2 is the stress at which a material exhibits 0.2% deviation from the proportionality of stress to strain. This figure, sometimes called "0.2% offset" is commonly used to measure the tensile strength and, indirectly, the tensile ductility of alloys such as ours.

As was stated before, the elements aluminum, titanium, boron and molybdenum are significant elements in determining the strength properties of nickel base alloys. Slight variations in percentages of these elements in alloys such as ours produce significant differences in physical

5

10

15

properties. Metallurgical technology along these lines has advanced to the point where it is no longer possible to broadly designate the composition range of such elements as aluminum, titanium, molybdenum and boron and still be able to predict the physical properties which will result. In addition, new important heat treatment cycles must be specified in order to control the precipitation of phases which are developed in alloys having aluminum, titanium, molybdenum and boron as part of their composition.

As an illustration, Table 3 includes the composition ranges and the average stress rupture life of a number of heats of material which we have prepared and tested. The stress rupture properties were obtained at 1800° F. with the samples under an axial load of 15,000 pounds per square inch:

Table 3

[Composition (percent by weight)]

| Ex.      | Avg.<br>Stress<br>Rupture<br>Life<br>(Hours) | C   | Fe  | Cr   | B   | Ti  | Al  | Mo  | Ni   | Si  | Mn  | S    |
|----------|----------------------------------------------|-----|-----|------|-----|-----|-----|-----|------|-----|-----|------|
| A-2----- | 94                                           | .05 | 4.8 | 15.6 | .09 | 2.1 | 4.6 | 4.0 | Bal. | .10 | .05 | .006 |
| A-3----- | 213                                          | .05 | 4.8 | 15.6 | .09 | 2.8 | 4.6 | 4.0 | Bal. | .10 | .05 | .005 |
| A-4----- | 290                                          | .05 | 4.8 | 15.0 | .09 | 3.5 | 4.6 | 4.0 | Bal. | .10 | .05 | .005 |
| G-3----- | 313                                          | .08 | 4.8 | 15.6 | .09 | 4.0 | 3.6 | 6.9 | Bal. | .06 | .05 | .006 |
| C-3----- | 543                                          | .05 | 4.7 | 15.2 | .08 | 3.5 | 4.4 | 5.3 | Bal. | .10 | .05 | .007 |
| C-1----- | 59                                           | .07 | 4.7 | 15.8 | .08 | 3.5 | 2.6 | 5.3 | Bal. | .10 | .05 | .007 |
| D-4----- | 446                                          | .07 | 4.8 | 14.8 | .08 | 2.7 | 4.5 | 5.4 | Bal. | .06 | .05 | .007 |

It is to be noted that the alloys of Examples A-4, G-3 and D-4, which lie within our unusual composition range, all have unusually high stress rupture lives at 1800° F. under an axial load such as 15,000 pounds per square inch. All the alloys shown in Table 3 were heat treated according to Example A of Table 6.

In Table 3 it can be seen that as the titanium content increases over a very narrow range, the stress rupture life increases over a very wide range thus showing the importance of such range. Similarly, small differences in aluminum content may result in vast differences in stress rupture life. This is easily seen by comparison of Examples C-3 and C-1. From the testing of a group of alloys of which the examples of Table 3 are a part, we found that the most significant range of molybdenum, titanium and aluminum in an alloy such as ours was in percent by weight molybdenum, 4-7, aluminum 3.6-5 and titanium 3-4. Of this range we prefer the range in percent by weight of molybdenum 4.5-6.0, aluminum 4.4-4.8 and titanium 3.25-3.65. The specific compositions which gave the most outstanding results are shown by Examples C-3 and D-4 of Table 3.

Although we had determined that a certain specific range for titanium, molybdenum and aluminum, coupled with the other elements in percent by weight of carbon .08 max., iron 4-6, chromium 14-17, boron about .05-.10 with the balance essentially nickel and impurities, we recognized in our testing that the average grain diameter of our alloy was another important factor in determining strength properties of alloys such as ours in cast form.

In a property evaluation program of this alloy, we noted that there was a variation in stress rupture lives which could not be explained either by chemical analysis or metallographic studies. However, we noted that there was a relationship between the average grain diameter and the stress rupture life in that increasing average grain diameter gave increasing stress rupture life. Our theory was statistically confirmed using the four quadrant correlation technique. This method, the results of which are shown in FIGURE 3, consists of dividing the plot into four quadrants by averaging abscissa values and ordinate values independently. The quadrants are then numbered consecutively counter-clockwise beginning with the upper right quadrant. Points falling in the quadrants I and III are designated positive and II and IV negative. FIGURE

3 shows 35 positive values as opposed to only 2 negative values indicating a strong positive correlation.

This correlation was further substantiated by the fact that four different heats of material were vacuum cast into different shapes and tested by different sources. The results of such varied materials show the correlation.

In order to produce grains of a controlled size, we first melted our alloy in a crucible and then cooled while still in a crucible to a temperature just above the solidification point, a point at which both solid and liquid are in equilibrium. Thus we formed small solid particles or nuclei in the melt. Then we applied full power to our equipment to raise the temperature of the melt as fast as possible. After a predetermined time, we poured or cast the metal from the crucible into a mold. The lapse of time between this latter increase in temperature of

Table 4

[Stress rupture properties at 1800° F. and 15,000 p.s.i.]

|       | Example | Stress<br>Rupture<br>Life (Hrs) | Average<br>Grain<br>Diameter<br>(Inches) |
|-------|---------|---------------------------------|------------------------------------------|
| 2852  |         | 623                             | 0.188                                    |
| X-920 |         | 551                             | 0.156                                    |
| 2851  |         | 482                             | 0.125                                    |
| X-930 |         | 421                             | 0.094                                    |
| X-900 |         | 273                             | 0.025                                    |
| X-923 |         | 94                              | 0.006                                    |
| X-921 |         | 91                              | 0.0035                                   |

The chemical analyses of the examples of Table 4 above are shown in the following Table 5:

Table 5

[Composition in percent by weight]

| Example | C    | S     | Al   | Ti   | Mo   | Cr   | Fe   | B     | Si   | Mn   |
|---------|------|-------|------|------|------|------|------|-------|------|------|
| 2-882   | 0.05 | 0.003 | 4.45 | 3.60 | 5.30 | 14.4 | 4.80 | 0.075 | 0.10 | 0.05 |
| X-920   | 0.05 | 0.004 | 4.40 | 3.65 | 5.55 | 14.6 | 4.55 | 0.081 | 0.10 | 0.10 |
| 2-851   | 0.04 | 0.006 | 4.35 | 3.40 | 5.35 | 14.3 | 4.60 | 0.080 | 0.10 | 0.05 |
| X-930   | 0.03 | 0.005 | 4.30 | 3.30 | 5.40 | 15.0 | 4.10 | 0.080 | 0.10 | 0.10 |
| X-900   | 0.05 | 0.004 | 4.37 | 3.33 | 5.25 | 14.7 | 4.50 | 0.076 | 0.07 | 0.05 |
| X-923   | 0.04 | 0.004 | 4.30 | 3.40 | 5.45 | 14.5 | 4.40 | 0.080 | 0.10 | 0.10 |
| X-921   | 0.06 | 0.005 | 4.30 | 3.45 | 5.40 | 14.5 | 4.55 | 0.088 | 0.10 | 0.10 |

the melt and the time of pouring determined the size of grains produced since that period is the initial factor which controls the growth of the grains. Other factors such as the size of the section being poured or the temperature of the mold bear a relationship to the ultimate grain size. The time required for melting equipment to produce grains of a given size will vary from unit to unit depending on its power capacity and the like. Therefore, the period of application of the last surge of power must be calibrated for each unit to produce grains of a given size.

The resultant grains tend to be regularly shaped, sometimes called "equi-axed grains" rather than elongated, rod-like grains sometimes referred to as "columnar grains."

The method which we used to measure average grain diameter and one which is highly reliable and reproducible is as follows: we first cut and polished a cross-section of a test bar normal to its longitudinal direction. After etching to distinguish grain structure, we then inscribed two perpendicular lines on that surface. We counted the number of grains in a measured length along one of the lines and divided that length by the number of grains counted. We then repeated the count for the other line and averaged the values together. For example, if five grains are found along one inch of the line, the average grain diameter would be  $\frac{1}{5}$  inch or 0.2 inch. The value thus obtained is the actual average grain diameter and not a reference number.

In FIGURE 3, the American Society for Testing Materials (ASTM) values are shown for comparison purposes along with our actual average grain diameter values. Therefore, the values for average grain diameter for our alloy which we have found produces increased stress rupture strength properties is greater in size than about ASTM macro-grain size number M-13 or about 0.015 inch. Preferably the average grain diameter of our alloy should lie within the range between about ASTM macro-grain size number M-6 and M-12 or about 0.02-0.25 inch.

As shown in Table 4, as average grain diameter decreases, stress rupture life decreases.

Although our alloy in the as-cast form exhibits unusual stress rupture properties, some of the heat treatment cycles which we studied led to our improving the stress rupture strength of our alloy even more over that of other currently available alloys. Table 6 gives examples of such cycles:

|   | Example: | Heat treatment cycle                                                                                                         |
|---|----------|------------------------------------------------------------------------------------------------------------------------------|
| A | -----    | heat at 2100° F. for 1 hour, air cool,<br>heat at 1950° F. for 2 hours, air cool,<br>heat at 1550° F. for 4 hours, air cool. |
| B | -----    | heat at 2100° F. for 1 hour, air cool,<br>heat at 1500° F. for 12 hours, air cool.                                           |
| C | -----    | heat at 2100° F. for 1 hour, air cool.                                                                                       |
| D | -----    | heat at 2200° F. for 1 hour, air cool,<br>heat at 1500° F. for 12 hours, air cool.                                           |
| E | -----    | heat at 1500° F. for 12 hours, air cool.                                                                                     |

The lengths of time referred to in Table 6 are the times at which the material being heat treated is in equilibrium with the temperature specified.

Although in general stress rupture strength decreases rapidly in excess of 1800° F., it has not been practical to conduct stress rupture testing at higher temperatures under an axial load of 15,000 p.s.i. However, the stress rupture properties of our alloy were so great that we were able to conduct stress rupture testings at 1850° F. under an axial load of 15,000 p.s.i. The results of stress rupture testing of a number of samples heat treated according to the heat treatments shown in Table 6 are shown in Table 7.

|   | Heat treatment: | Average stress rupture life (hours) |
|---|-----------------|-------------------------------------|
| A | -----           | 153                                 |
| B | -----           | 190                                 |
| C | -----           | 200                                 |
| D | -----           | 189                                 |
| E | -----           | 96                                  |

Referring to Table 7, it is to be noted that an initial heating or solution-heat treating at about 2100-2200° F.

will produce relatively high stress rupture properties. The heat treatment which we found best is shown as heat treatment C. It involves only the heating at about 2100° F. for one hour and then air cooling. Most other commercially available high temperature alloys will require the use of a commercial furnace for approximately one day or longer in order to complete their heat treatment cycles sometimes referred to as "double aging cycles." The introduction of a heat treatment cycle such as shown in Example C of Table 6 to give exceedingly high stress rupture properties reduces the cost of the manufacture of articles by a substantial amount.

Although in the foregoing description we have disclosed in connection with specific examples an improved precipitation hardening type nickel base alloy and heat treatment for such alloy to produce stress rupture strength properties in excess of any nickel base alloys heretofore produced, the examples are to be construed as illustrative of rather than limitations on our invention. Those skilled in the art of metallurgy and heat treatment will readily understand the modifications and variations of which our invention is capable. We intend in the appended claim

to cover modifications and variations which come within the true spirit and scope of our invention.

What we claim as new and desire to secure by Letters Patent of the United States is:

A precipitation hardening type nickel base alloy suitable for use at elevated temperatures consisting of, by weight, 0.05% carbon, 4.1-4.8% iron, 15% chromium, 3.5% titanium, 0.08% boron, 4.5% aluminum, 5.3% molybdenum, with the balance essentially nickel and impurities; the alloy having an average grain diameter of 0.02-0.25 inch.

References Cited in the file of this patent

FOREIGN PATENTS

502,822 Italy ----- Dec. 1, 1954  
769,822 Great Britain ----- Mar. 13, 1957

OTHER REFERENCES

Metallic Creep and Creep Resistant Alloys, A. H. Sully, Interscience Publishers Inc., New York, 1949, p. 128 relied upon, copy in Sci. Lib.